

## UNITED STATES PATENT OFFICE

GUSTAVE S. MATHEY, OF ELIZABETH, NEW JERSEY, ASSIGNOR TO JOHNSON & JOHNSON, OF NEW BRUNSWICK, NEW JERSEY, A CORPORATION OF NEW JERSEY

## TENNIS STRING

No Drawing.

Application filed July 9, 1927. Serial No. 204,667.

The ever increasing cost of gut has resulted in appreciable decline in its use as the raw material in the manufacture of tennis racket strings and the like. Nevertheless, no satisfactory substitute has heretofore been devised.

The silk strings of commerce undoubtedly will outwear almost any grade of gut string but they have a lower order of resiliency or 10 liveliness. To some extent the advantages and disadvantages of steel strings are similar to those of silk. Whether covered or not, steel strings are less lively than gut and steel strung rackets have a different "feel".

15 There are on the market at present only a few synthetic strings. Braided strings are rapidly disappearing. A few special strings, combining gut and silk, have been offered, but their disadvantages over-shadow any 20 apparent advantages.

The silk string offers the best solution provided it can be improved as to resiliency and as to waterproof properties.

After extended experimentation with 25 many raw materials and divers methods of fabrication and treatment, I have devised a comparatively low cost strand which practically equals the resiliency of gut and for durability and over all efficiency is far superior to gut. It possesses the further merit 30 that in appearance it is almost identical with gut in that it is substantially transparent, a cross-section of the string revealing no fibrous structure. And the new strand may 35 be untwisted with even more difficulty than is the case with gut strings.

In the practice of my invention, I start with silk in the boiled-off condition, i. e. free from the silk gum, ceresin. The elimination 40 of ceresin is highly important for I have found that the presence of this substance is a deterrent to successful impregnation and accounts for past failures. A size of silk which has proven satisfactory is 22 thread 45 13/15 Japan tram.

Having, as stated, completely removed all traces of ceresin, the strands of silk are twisted and drawn under desirable tension through an appropriate glue mixture which 50 is held at a carefully regulated temperature.

In general, the higher the temperature, the better the impregnation. However, it is not desirable to raise the temperature of the glue appreciably beyond 70° C., otherwise hydrolysis of the glue takes place and the finished string is likely to be decidedly brittle.

55

The temperature is regulated according to the fluidity of the glue and the appearance of the twisted string.

As a result of testing a number of types of 60 cementing agents such as glass, resins, varnishes, lacquers, etc., I have found that a true colloid in solid form to the jelly form results in a true colloid jelly which shrinks uniformly and dries without any separation from 65 the strands.

In those tests in which varnishes or lacquers were used, it was found that the resulting strings were quite large, poorly impregnated, slow in drying, and not at all satisfactory as tennis strings.

70

Flexibility in the finished string is essential, otherwise the string will almost certainly break at the frame in the stringing process. The desired flexibility may be obtained by 75 the use of a satisfactory softening agent in the glue mixture. However, the use of such agent in the required amount tends to confer upon the string a resin-like surface so that when the string is pulled through a racket 80 form it slips at intervals as though it were treated with pine resin. Obviously, this condition is altogether undesirable inasmuch as it makes for non-uniformity of tension. To overcome this action of the softening agent, I 85 add a good lubricant such as castor oil, lard or other vegetable or animal product. Good results have also been had with petroleum oils. The oil is stirred into the glue mixture until a uniform emulsion is formed in which 90 no trace of oil may be observed. Such an emulsion may be kept almost indefinitely with no separation into its components and possesses many of the properties of the simple 95 glue mixture. The use of emulsions of this type has been found to insure satisfactory strings capable of withstanding the roughest treatment.

Typical glue mixtures which yield quite 100

satisfactory products are given in the accompanying table,

|              |    |    |    |    |    |
|--------------|----|----|----|----|----|
| Glue         | 30 | 30 | 30 | 25 | 25 |
| Glycerin     | 20 | 15 | 15 | 15 | 10 |
| 5 Castor oil | 20 | -- | -- | -- |    |
| Lard         | -- | 20 | 25 | 30 |    |
| Water        | 50 | 35 | 35 | 35 |    |

It will be noted that the composition of the glue mixture or emulsion may be varied over rather wide limits according to the characteristics desired in the product. Other softening agents such as glycol, diethylene glycol, triethylene glycol, the various poly-glycerins, etc., may be substituted for the glycerin used in the present process, and various oils of almost any origin may be substituted for the lard.

The properties of the finished string depend largely upon its structure. A twisted string having from two to four twists to the inch, and preferably a twist of three turns to the inch, has proven eminently satisfactory.

A string containing glue as such is not water-proof. By proper treatment, however, the glue may be rendered very resistant to the action of moisture. The common tanning agents for leather are in general capable of rendering glue moisture-proof. Among these are formaldehyde, other aldehydes, hexamethylene tetramine, tannic acid, potassium dichromate, and chromium and aluminum salts. From the standpoint of ease of handling, low price and results obtained, formaldehyde has been most satisfactory. As carried out at present, curing is obtained by exposing the twisted string to the vapor of formaldehyde in a closed environment. The use of solutions of formaldehyde containing the softening agent used in the glue mixture has also proved satisfactory.

After removal from the curing vessel the strings are stretched tightly and allowed to remain until dry. The quality of the strings is improved somewhat if the drying is conducted under considerable tension.

After the strings are thoroughly dried, any small surface irregularities may be removed by polishing with sand paper or equivalent, whereupon the strings are wiped off with lard or other oil.

A satisfactory string must possess a breaking strength of not less than one hundred pounds straight pull. This strength is insured in the string of the instant case by the use of between fifty or sixty strands of 22 thread 13/15 Japan tram.

Strings of a solid color may be provided by simply adding the desired color to the emulsion or glue mixture. Where more than one color is required, the use of two or more kinds of colored silk will insure the desired combination of colors.

While the present product is mainly intended for use as a substitute for gut it is

well qualified or may readily be qualified for other purposes by modifying the glue bath, by proper choice of capillary bore or other trim, and/or by varying the number of strands. For example it may replace raw 70 hide in hookless belt lacing.

Having described my invention, I claim:

A synthetic gut, comprising twisted strands of degummed silk, and an emulsified colloidal bond having lubricating and water-proofing properties.

In testimony whereof I affix my signature.

GUSTAVE S. MATHEY.

80

85

90

95

100

105

110

115

120

125

130